

# UNITED STATES PATENT OFFICE.

JOHN E. SPRINGER, OF NORFOLK, VIRGINIA.

## ALLOY.

1,413,880.

Specification of Letters Patent. Patented Apr. 25, 1922.

No Drawing.

Application filed August 13, 1920. Serial No. 403,268.

To all whom it may concern:

Be it known that I, JOHN E. SPRINGER, a citizen of the United States, and resident of Norfolk, in the county of Norfolk and State 5 of Virginia, have invented certain new and useful Improvements in Alloys, of which the following is a specification.

My invention relates to improvements in alloys or compounds, and it consists sub- 10 stantially in the ingredients and proportions thereof, as herein specified and claimed.

One of the foremost objects sought to be accomplished by this particular compound, is to produce a metallic alloy possessing the 15 important advantages of lightness, strength, ductility and relative cheapness. The alloy is composed of the following ingredients:

|    |                   |     |
|----|-------------------|-----|
|    | Furnace slag----- | 50% |
| 20 | Humite-----       | 8%  |
|    | Copper-----       | 20% |
|    | Nickel-----       | 5%  |
|    | Zinc-----         | 5%  |
|    | Tungsten-----     | 5%  |
| 25 | Iron-----         | 2%  |
|    | Manganese-----    | 5%  |

In making a batch or quantity of the alloy, all of the above ingredients are taken at once and placed in a furnace, being there 30 heated to a melting temperature. The furnace slag and humite act as fluxes which aid the commingling of the metallic elements in producing the final alloy. The molten mass is poured into a flask or mold. After 35 the article has cooled it is heat treated or annealed, which treatment, as is commonly known, consists merely in bringing the article to a predetermined temperature and then again permitting it to cool.

40 The above schedule gives the proportions of the ingredients in percentages. From

this it is an easy matter to compute the relative weights of the various ingredients for any desired total weight of alloy. All of the ingredients are familiar but humite may 45 be identified as a mineral of the chondrodite variety, crystalline and translucent, brownish-yellow to white in color, composed of magnesia, silicia, fluorine, and protoxide of iron.

The alloy is rust-proof, non-corrosive and does not deteriorate. The uses to which it can be put are many, a few being here stated; it may be made into telegraph poles, rail road ties, lintels, roofing plates, paving 55 blocks, sheet piling, etc. When roofing plates are made, the material is cast in sheets approximating the ordinary thickness of slate shingles.

Since the alloy possesses the quality of 60 ductility, such plates may be readily shaped to any form desired. A special application of the alloy is that to making railroad ties, in which case the ties are made hollow.

I claim:

1. The herein described method of making an alloy consisting of taking the following metallic ingredients and proportions thereof; copper 20%, nickel 5%, zinc 5%, tungsten 5%, iron 2%, manganese 5% and the 70 fluxes furnace slag 50%, humite 8%; heating all ingredients together to a melting temperature molding the resultant alloy, and annealing it.

2. The herein described alloy comprising 75 the following ingredients and proportions thereof remaining after melting with the fluxes furnace slag 50% and humite 8%, copper 20%, nickel 5%, zinc 5%, tungsten 5%, iron 2%, manganese 5%.

JOHN E. SPRINGER.